

Feb. 10, 1959

F. G. FOOTE

2,873,186

THORIUM-SILICON-BERYLLIUM ALLOYS

Filed June 9, 1948



INVENTOR.

Frank Foote

BY

Roland A. Anderson

Attorney

## 1

2,873,186

**THORIUM-SILICON-BERYLLIUM ALLOYS**

Frank G. Foote, Plandome, N. Y., assignor to the United States of America as represented by the United States Atomic Energy Commission

Application June 9, 1948, Serial No. 31,923

5 Claims. (Cl. 75—122.7)

This invention relates to alloys of thorium and more particularly to alloys wherein thorium metal is alloyed with more than one other element.

An object of this invention is to provide an alloy of thorium having improved physical properties, namely, increased resistance to corrosion and improved hardness values.

A further object of this invention is to provide an alloy of thorium containing certain added elements to impart special properties to the thorium metal wherein these special properties are increased to a degree beyond that ordinarily expected to result from the addition of equal or even greater amounts of either of the minor alloying elements alone.

Other objects and advantages will be apparent to those skilled in the art upon further examination of this specification and the accompanying drawing which is the thorium corner of the phase diagram for the ternary system comprising thorium, silicon and beryllium.

In accordance with this invention, it has been discovered that the simultaneous use of both silicon and beryllium as alloying elements with thorium produces an alloy having physical properties at least comparable or even superior to those found in the binary thorium alloys containing either beryllium or silicon alone. Moreover, it appears that the simultaneous use of both silicon and beryllium in a thorium alloy produces a synergistic effect in that the sum of the amounts of both silicon and beryllium used in combination with each other is less than the amount of either of the alloying elements used singly to produce a thorium alloy having identical or improved properties.

The ternary alloys of thorium, silicon and beryllium show increased hardness values and a greater resistance to aqueous corrosion than is found in pure thorium metal or in either binary alloy consisting of thorium-silicon or thorium-beryllium. On account of these improved physical properties and because of their characteristics suitable for nuclear bombardment processes, these ternary alloys are well adapted for use in construction of water-cooled chain-reacting piles.

The subject matter of this invention includes those

## 2

ternary alloys consisting primarily of thorium metal alloyed with both beryllium and silicon, the amount of each of said minor alloying elements being between 0.1 and 3.5% by weight, wherein the minimum total

5 weight percent of silicon and beryllium is 1.5, the maximum total weight percent of said minor alloying elements is 4.5% and the balance is substantially pure thorium. Such alloys have improved physical characteristics over those found in thorium metal or either of the binary 10 alloys of thorium containing silicon or beryllium alone. These limits for compositions of matter within the purview of this invention are shown in the drawing by the heavy solid lines.

Upon further investigation of the thorium corner of 15 the phase diagram for the three-component system, it has been discovered that thorium alloyed with between 0.4 and 3.0% by weight beryllium and between 0.3 and 3.0% by weight silicon wherein the total weight percent of minor alloying elements is between 1.5 and 20 4.0% by weight constitutes a preferred range for each of the elements present. The limits of the preferred compositions of matter are designated by the broken lines and the solid line joining the broken lines for compositions containing 1.5% total beryllium and silicon. 25 Stated in terms of percent of thorium, such total weight percents of minor alloying elements necessarily implies alloys containing between 96.0 to 98.5 weight percent thorium. These alloys containing thorium, silicon and beryllium within the above ranges show increased hardness values as follows:

| Percent<br>Silicon by<br>Weight | Percent<br>Beryllium<br>by Weight | Cast Hardness<br>Rockwell "B"<br>Scale |
|---------------------------------|-----------------------------------|----------------------------------------|
| 0.62                            | 1.11                              | 89                                     |
| 1.65                            | 0.52                              | 93                                     |
| 1.64                            | 1.05                              | 94                                     |

35 40 whereas an alloy having a composition outside the preferred area, e. g. 0.64 and 0.44 weight percent for silicon and beryllium respectively, shows a cast hardness of only 69 on the Rockwell "B" scale.

Increased resistance to aqueous corrosion as well as 45 improved hardness values is shown by those ternary compositions consisting of thorium metal alloyed with between 1.0 and 1.5% by weight beryllium and between 0.5 and 1.0% by weight silicon wherein the total weight percent of said minor alloying elements is between 1.5 and 2.0% by weight.

The following tabulated data demonstrate the superior resistance to corrosion and hardness found in the ternary alloys in comparison to the binary thorium-silicon and thorium-beryllium alloys.

TABLE I  
Corrosion of thorium alloys in water (178° C.)  
(autoclave tests)

| Nominal Wt. Percent Alloy<br>Element                        | Cast Hardness<br>Values<br>on Rockwell<br>"B" Scale | Weight Change (mg./cm. <sup>2</sup> ) Based on Uncleaned Specimens |          |                  |        |         |         |
|-------------------------------------------------------------|-----------------------------------------------------|--------------------------------------------------------------------|----------|------------------|--------|---------|---------|
|                                                             |                                                     | 0.8 day                                                            | 1.7 days | 4 days           | 8 days | 16 days | 32 days |
| Thorium.....                                                | 52                                                  | 0.47                                                               | 0.00     | -0.04            | -12.3  | -94.3   | -248    |
| Th+1.08 wt. Percent Si.....                                 | 68                                                  | 0.51                                                               | 0.69     | 1.0              | -39.2  | -171    | -495    |
| Th+2 wt. Percent Si.....                                    | 75                                                  | 0.20                                                               | 0.26     | 1.0              | -9.3   | -106    | -339    |
| Th+4.3 wt. Percent Si.....                                  | 88                                                  | 0.0                                                                | -0.28    | 0.03             | -12.3  | -74     | -249    |
| Th+<br>0.62 wt. Percent Si.....<br>1.11 wt. Percent Be..... | 89                                                  | -0.58                                                              | -1.0     | -0.96            | -0.83  | -3.8    | +0.4    |
| Th+0.4 wt. Percent Be.....                                  | 84                                                  | 0.46                                                               | 1.7      | 1.65             | 5.0    | 7.0     | +28     |
| Th+0.94 wt. Percent Be.....                                 | 68                                                  | 0.32                                                               | -0.13    | ( <sup>1</sup> ) | -      | -       | -       |
| Th+2.46 wt. Percent Be.....                                 | 87                                                  | -0.55                                                              | -1.2     | -1.1             | -0.97  | -0.6    | -0.7    |

<sup>1</sup> Completely corroded.

TABLE II

*Corrosion rates of pure Th, Th-exploratory alloy binary systems, and Th-Si-Be ternary in boiling distilled H<sub>2</sub>O<sup>+</sup>*

| Weight Percent of Alloy Material | Heat Treatment      | Cast Hardness on Rockwell "B" Scale | Hours of Test | Wt. Change, mg./cm. <sup>2</sup> /hr. |
|----------------------------------|---------------------|-------------------------------------|---------------|---------------------------------------|
| Pure Thorium                     | Extruded            | 52                                  | 852           | -.003                                 |
| 0.49 Beryllium                   | Cast from 1,355° C  | 84                                  | 112           | +.005                                 |
| 0.94 Beryllium                   | Cast from 1,350° C  | 68                                  | 112           | +.008                                 |
| 1.6 Beryllium                    | Cast (BeO crucible) | 68                                  | 112           | +.0023                                |
| 2.46 Beryllium                   | Cast from 1,330° C  | 87                                  | 112           | +.003                                 |
| 1.08 Silicon                     | Cast from 1,755° C  | 68                                  | 112           | +.002                                 |
| 2.0 Silicon                      | Cast from 1,660° C  | 75                                  | 112           | +.002                                 |
| 4.3 Silicon                      | Cast from 1,670° C  | 88                                  | 112           | +.002                                 |
| 0.62 Silicon; 1.11 Beryllium     | Cast from 1,330° C  | 89                                  | 112           | +.001                                 |

The thorium-silicon eutectic occurs at approximately 2% by weight silicon and melts above 1300° C. whereas the eutectic for the binary thorium-beryllium alloy occurs at approximately 2% by weight beryllium and melts between 1100 and 1200° C. The two eutectics are connected by an eutectic valley sloping from a maximum at the thorium-silicon eutectic to a minimum at or very close to the thorium-beryllium eutectic.

By examination of the microstructures of the alloys defined by the subject matter of this invention it appears that the ternary alloys consisting of thorium, beryllium and silicon are, in reality, mixtures of the binary eutectics. Samples of these binary and ternary alloys were etched electrolytically in phosphoric acid solution prior to examination of the microstructures.

The binary-thorium-silicon eutectic occurring at 2% by weight silicon appears as a coarse eutectic made up of gray particles. The binary thorium-beryllium eutectic, also containing about 2% by weight of the minor alloying element, beryllium, appears as an extremely fine herringbone type upon examination of the microstructure.

The ternary eutectic does not have an easily recognized microstructure and the ternary alloys in the vicinity of the eutectic valley show these binary eutectics as they appear in the binary alloys, neither altering the appearance of the other.

For example, the ternary alloy, wherein 1.05% by weight beryllium and 1.64% by weight silicon is alloyed with thorium, appears to consist primarily of a coarse silicon eutectic mixed with a small amount of the extremely fine beryllium eutectic. Where thorium is alloyed with 1.11% by weight beryllium and 0.62% by weight silicon, the microstructure reveals large amounts of both the coarse-grained silicon-thorium eutectic and the fine herringbone type beryllium eutectic, and in this structure the quantitative relationship between the two types of eutectic mixtures was not quite so marked.

It will be apparent to those skilled in the art to which this invention pertains that various modifications may be made without departing from the principles of

the invention as disclosed herein, and thus it is not intended that the invention should be limited other than by the scope of the appended claims.

What is claimed is:

1. An alloy consisting essentially of thorium, silicon and beryllium.
2. An alloy consisting essentially of thorium as the predominant ingredient and minor quantities of silicon and beryllium.
3. An alloy consisting of thorium, silicon and beryllium wherein beryllium and silicon are each present in amounts between 0.1 and 3.5% by weight and the total weight percent of said minor alloying elements is between 1.5 and 4.5, and the balance is substantially thorium.
4. An alloy consisting of thorium, silicon and beryllium wherein the beryllium present is between 0.4 and 3% by weight and the silicon present is between 0.3 and 3.0% by weight, and the total weight percent of said minor alloying elements is between 1.5 and 4.0.
5. An alloy consisting of thorium, silicon and beryllium wherein the hardness values range upwards from 75 on the Rockwell "B" scale and there is improved resistance to corrosion in the cast alloy containing beryllium between 1.0 and 1.5% by weight and silicon between 0.5 and 1.0% by weight, and the total weight percent of said minor alloying elements is between 1.5 and 2.0% and the remainder is predominantly thorium.

#### References Cited in the file of this patent

##### UNITED STATES PATENTS

1,602,526 Gerö ----- Oct. 12, 1926

##### FOREIGN PATENTS

258,642 Great Britain ----- Sept. 20, 1926

##### OTHER REFERENCES

Goodman: The Science and Engineering of Nuclear Power, p. 364 (1947), publ. by Addison-Wesley Press, Cambridge, Mass.